# EUROPEAN PATENT SPECIFICATION

(11) **EP 3 395 987 B1**
(45) Date of publication and mention of the grant of the patent: **29.04.2020**
(21) Application number: 16879393.3
(22) Date of filing: 23.12.2016
(51) Int. Cl.: C22C 38/14, C22C 38/12, C22C 38/08, C22C 38/06, C22C 38/04, C22C 38/02, C21D 8/02, C21D 6/00

(54) **LOW-YIELD RATIO AND HIGH-STRENGTH STEEL HAVING EXCELLENT STRESS CORROSION CRACKING RESISTANCE AND LOW TEMPERATURE TOUGHNESS**
HOCHFESTE STAHLPLATTE MIT NIEDRIGER STRECKGRENZE UND AUSGEZEICHNETER SPANNUNGSRISSKORROSIONSBESTÄNDIGKEIT UND NIEDRIGER TEMPERATURZÄHIGKEIT
ACIER À HAUTE RÉSISTANCE ET À FAIBLE TAUX D'ÉLASTICITÉ PRÉSENTANT UNE EXCELLENTE RÉSISTANCE À LA FISSURATION PAR CORROSION SOUS CONTRAINTE ET UNE EXCELLENTE TÉNACITÉ À BASSE TEMPÉRATURE

(30) Priority: 23.12.2015 KR 20150185496
(43) Date of publication of application: 31.10.2018
(73) Proprietor: POSCO, Nam-gu Pohang-si, Gyeongsangbuk-do 37859 (KR)
(72) Inventor: JANG, Sung-Ho, Pohang-si, Gyeongsangbuk-do 37877 (KR); LEE, Hak-Cheol, Pohang-si, Gyeongsangbuk-do 37877 (KR)
(74) Representative: Potter Clarkson
(86) International application number: PCT/KR2016/015156
(87) International publication number: WO 2017/111526

(56) References cited:
- EP-A1- 2 940 172
- WO-A1-2009/072753
- JP-A- 2009 127 065
- JP-A- 2012 107 310
- JP-A- 2012 107 310
- KR-A- 20110 075 627
- KR-A- 20110 116 760
- KR-A- 20130 110 643
- KR-A- 20130 110 643
- KR-A- 20140 023 787

## Description

### [Technical Field]

The present disclosure relates to a low yield ratio and high-strength steel having excellent stress corrosion cracking resistance and low temperature toughness.

### [Background Art]

Although varied according to types of a liquefied gas, a temperature for liquefying a gas is generally low (-52°C in the case of LPG) at normal pressure, and thus, steel used in a liquefied gas storage tank has been required to have excellent low temperature toughness in a welded part, as well as in a base material.

It is known that liquid ammonia (LAG) causes stress corrosion cracking (SCC) of steel, and thus, IGC CODE (International Code for the Construction and Equipment of Ships Carrying Liquefied Gases in Bulk) regulates operating conditions at the time of manufacturing, such as oxygen partial pressure, temperature, and the like, limits the Ni content of steel to 5% or less, and defines actual yield strength to 440 MPa or less.

In addition, when a gas tank is manufactured by welding steel for a gas tank, removal of stress from a welded part is an important consideration. Therefore, methods for removing stress from a welded part include a post welding heat treatment (PWHT) based on a heat treatment and a mechanical stress relief (MSR) method of removing stress by adding hydrostatic pressure, or the like, to the welded part, or the like. In the case of removing stress from the welded part using the mechanical stress relieving (MSR) method, deformation is applied to a base material part due to water pressure, and thus, a yield ratio of the base material is limited to 0.8 or less. Here, in removing stress using MSR, if deformation equal to or greater than yield strength is applied to the base material part due to high pressure water injection, if a ratio of the yield strength and tensile strength is high, yield occurs, that is, tensile strength may be reached to cause damage, and thus, yield strength and tensile stress are limited, to be significantly different.

In particular, since gas tanks are basically required to be enlarged in size, it may be difficult to remove stress by the PWHT method and most shipbuilders prefer the MSR method, and thus, steel for manufacturing gas tanks is required to have low yield ratio characteristics.

In this manner, in the tanks in which the LPG and the LAG coexist, it is a significant issue to achieve both low temperature toughness and a low yield ratio accompanying the regulation of an upper limit of yield strength from liquid ammonia.

Meanwhile, Patent document 1 proposes a technique of adding 6.5 to 12.0% of Ni to achieve excellent low temperature toughness. Also, Patent document 2 proposes a technique of mixedly using tempered martensite and bainite by performing quench tempering on steel having a specific composition.

However, in general, if a large amount of Ni is added, a large amount of austenite phases having an FCC lattice structure, which is easily deformed due to a narrow interatomic gap, may be formed, and if repeated stress and a corrosive environment are applied to the easily deformed FCC lattice structure, corrosion may easily occur to cause cracking. Therefore, Patent document 1 has a problem of low economical efficiency due to high-priced Ni content and has a problem of degrading stress corrosion cracking (SCC) resistance.

Further, Patent document 3 proposes a technique of only softening a surface layer of a steel sheet to realize a low-yield ratio. This technique, however, may achieve low temperature toughness and low yield ratio separately but cannot obtain both low temperature toughness and low yield ratio together.

Meanwhile, in order to enhance strength of steel as another characteristic required for the steel, precipitation strengthening, solid solution strengthening, and martensite strengthening may be used but these methods degrade toughness and elongation, while enhancing strength.

In addition, in the case of increasing strength by refining crystal grains by applying various manufacturing conditions, high strength may be obtained and a degradation of toughness may be prevented due to a reduction in an impact toughness transition temperature. However, yield strength based on grain refinement may be increased to exceed 440 MPa, a yield strength upper limit, at which ammonia stress corrosion (SCC) occurs, and it is difficult to obtain low-yield ratio.

Therefore, there is a need to develop a low yield ratio and high-strength steel having excellent stress corrosion cracking resistance and low temperature toughness and a manufacturing method thereof

### <Related art document>

(Patent document 1) Patent document 1: Japanese Patent Laid-Open Publication No. S63-290246
(Patent document 2) Patent document 2: Japanese Patent Laid-Open Publication No. S58-153730
(Patent document 3) Patent document 3: Japanese Patent Laid-Open Publication No. H4-17613

WO2009072753 discloses a high-strength steel plate having acicular ferrite and bainite as a main microstructure and an austenite/martensite (M & A) as a second phase under the control of a cooling rate above the austenite transformation temperature. The high-strength steel plate comprises: carbon (C) : 0.03 to 0.10 wt%, silicon (Si): 0.1 to 0.4 wt%, manganese (Mn): 1.8 wt% or less, nickel (Ni): 1.0 wt% or less, titanium (Ti): 0.005 to 0.03 wt%, niobium (Nb): 0.02 to 0.10 wt%, aluminum (Al): 0.01 to 0.05 wt%, calcium (Ca) : 0.006 wt% or less, nitrogen (N): 0.001 to 0.006 wt%, phosphorus (P): 0.02 wt% or less, sulfur (S): 0.005 wt% or less, and the balance of iron (Fe) and other inevitable impurities . The method for manufacturing a high-strength steel plate may be useful economically and effectively to manufacture a high strength steel, which is able to secure excellent properties such as high strength and high toughness since the acicular ferrite and bainite may be effectively formed without adding expensive elements such as molybdenum (Mo).

EP2940172 A1 discloses a high strength steel sheet having low yield ratio properties and cryogenic temperature toughness and that are suitable to be applied to the steel material for a gas tank used for the storage of gas or the like.

### [Disclosure]

### [Technical Problem]

An aspect of the present disclosure is to provide a low yield ratio and high-strength steel having excellent stress corrosion cracking resistance and low temperature toughness, and a manufacturing method thereof.

Meanwhile, the aspect of the present disclosure is not limited to the above description. It will be understood by those of ordinary skill in the art that there is no difficulty in understanding the additional problems of the present disclosure.

### [Technical Solution]

The above mentioned problems are solved by providing a low yield ratio and high-strength steel excellent stress corrosion cracking resistance and low temperature toughness and its manufacturing method as disclosed in claims 1 to 9.

The foregoing technical solutions do not fully enumerate all of the features of the present invention. The foregoing and other objects, features, aspects and advantages of the present invention will become more apparent from the following detailed description of the present invention when taken in conjunction with the accompanying drawings.

### [Advantageous Effects]

As set forth above, according to an exemplary embodiment in the present disclosure, by controlling an alloy composition and microstructure, the low yield ratio and high-strength steel having excellent stress corrosion cracking resistance and low temperature toughness and the manufacturing method thereof may be provided.

### [Description of Drawings]

FIG. 1 is a view illustrating phase transformation of inventive steel A according to a cooling rate.
FIG. 2 is a photograph (1-(1) in FIG. 1) obtained by observing a microstructure of the 1/4t portion of a steel sheet of A-5 as comparative example with an optical microscope.
FIG. 3 is a photograph (1-(2) in FIG. 1) obtained by observing a microstructure of the 1/4t portion of a steel sheet of A-1 as inventive example with an optical microscope.
FIG. 4 is a photograph (1-(3) in FIG. 1) obtained by observing a microstructure of the 1/4t portion of a steel sheet of A-6 as comparative example with an optical microscope.

### [Best Mode for invention]

Hereinafter, preferred embodiments of the present disclosure will be described. However, the embodiments of the present disclosure may be modified into various other forms, and the scope of the present disclosure is not limited to the embodiments described below. Embodiments of the present invention are provided so that those skilled in the art may more completely understand the present invention.

The inventors of the present application recognized that it is difficult to make both ammonia stress corrosion cracking resistance and low temperature toughness excellent and have studied to solve the problem.

As a result, the inventors confirmed that it is possible to provide a low yield ratio and high-strength steel having excellent stress corrosion cracking resistance and low temperature toughness by controlling an alloy composition and a microstructure and a manufacturing method thereof, thereby completing the present disclosure.

First, an alloy composition of the low yield ratio and high-strength steel having excellent stress corrosion cracking resistance and low temperature toughness according to an aspect of the present disclosure will be described in detail. Hereinafter, the content of each component refers to weight percent (wt%).

### C (carbon): 0.02 to 0.10%

Since C is the most important element for securing basic strength, it is necessary to be contained within an appropriate range in the steel, and in order to obtain an additive effect, preferably, C is added in an amount of 0.02% or more.

If the C content is less than 0.02%, strength may be reduced and the yield ratio may be lowered, which is not preferable. If the C content exceeds 0.10%, a large amount of low temperature transformation phases such as bainite, or the like, is generated to exceed an upper limit of yield strength that may cause ammonia stress corrosion cracking (SCC).

Therefore, the content of C is limited to 0.02 to 0.10%. Preferably, it is 0.05 to 0.08%.

### Si (silicon): 0.05 to 0.5%

Si has an effect of increasing strength due to the effect of solid solution strengthening and is advantageously used as a deoxidizing agent in steel making process.

If the Si content is less than 0.05%, the deoxidation effect and the strength improving effect may be insufficient. If the Si content exceeds 0.5%, the low-temperature toughness is lowered and weldability is deteriorated.

Therefore, the silicon content is limited to 0.05 to 0.5%. Preferably, it is 0.05 to 0.3%.

### Mn (manganese): 0.5 to 2.0%

Manganese contributes to ferrite grain refinement and is an element useful for improving strength by solid solution strengthening.

In order to obtain the effect of manganese, manganese is required to be added in an amount of 0.5% or more. If, however, the content exceeds 2.0%, hardenability may be excessively increased, which promotes formation of upper bainite and martensite to significantly reduce impact toughness and ammonia stress corrosion cracking (SCC) resistance and to reduce toughness of weld heat-affected zone as well.

Therefore, the Mn content is limited to 0.5 to 2.0%. Preferably, it is 1.0 to 1.5%.

### Ni (nickel): 0.05 to 1.0%

Ni is an important element for facilitating cross slip of dislocations at low temperatures to improve impact toughness and hardenability and to improve strength. In order to obtain such an effect, Ni is preferably added in an amount of 0.05% or more. If the Ni content exceeds 1.0%, ammonia stress corrosion cracking (SCC) may occur and manufacturing costs may be increased due to the high cost of Ni relative to other hardenable elements.

Therefore, the Ni content is limited to 0.05 to 1.0%, and preferably, 0.2 to 0.5%.

### Nb (niobium) : 0.003% or less

It is known that Nb dissolved in reheating at high temperatures is precipitated very finely in the form of NbC to inhibit the recrystallization of austenite, thereby making the structure finer.

Since yield strength may be excessively increased due to microstructure refining, which may exceed the upper limit of yield strength that may cause ammonia stress corrosion cracking (SCC), Nb is controlled to 0.003% or less.

### Ti (titanium): 0.005 to 0.1%

Titanium forms oxides and nitrides in the steel to inhibit growth of crystal grains during reheating, thereby significantly improving low temperature toughness, and is also effective in refining the microstructure of a welded portion.

In order to obtain such an effect, titanium needs to be added in an amount of 0.005 wt% or more. If the content exceeds 0.1 wt%, low temperature toughness may be reduced due to clogging of a nozzle or crystallization of a central portion.

Therefore, the titanium content is 0.005 to 0.1%. Preferably, it is 0.01 to 0.03%.

### Al (aluminum): 0.005-0.5%

Aluminum is an element useful for deoxidizing molten steel, and to this end, aluminum needs to be added in an amount of 0.005 wt% or more. If the content exceeds 0.5 wt%, nozzle clogging may occur during continuous casting. Therefore, the aluminum content is 0.005 to 0.5%. Preferably, it is 0.005 to 0.05%.

### P (phosphorus): 0.015% or less

Phosphorus is an element that causes grain boundary segregation in a base material and a welded portion. Since phosphorus causes a problem of embrittling steel, an amount of phosphorus needs to be actively reduced. However, reducing phosphorus to an extreme limit may deepen a load of a steel making process and since the aforementioned problem does not significantly arise as long as the content of phosphorus is 0.015% or less, an upper limit thereof is limited to 0.015%, more preferably, to 0.010%.

### S (sulfur): 0.015% or less

Sulfur (S), an element which causes red shortness, forms MnS, or the like, to significantly inhibit impact toughness. Therefore, sulfur is preferably controlled to as low as possible and the content is limited to 0.015 wt% or less, more preferably, to 0.005 wt%.

The balance of the present disclosure is iron (Fe) . However, in the ordinary manufacturing process, impurities may be inevitably incorporated from a raw material or a surrounding environment, which may not be excluded. These impurities are known to any one skilled in the art in the ordinary manufacturing process and thus not specifically mentioned in this disclosure.

Next, a microstructure of the low yield ratio and high-strength steel having excellent stress corrosion cracking resistance and low temperature toughness according to one aspect of the present disclosure will be described in detail.

The microstructure of the steel of the present disclosure includes, in area %, 60% or more of acicular ferrite and a balance of at least one phase of bainite, polygonal ferrite and martensite-austenite constituent (MA).

If a fraction of the bainite is increased so the acicular ferrite is less than 60%, impact toughness may deteriorate due to an increase in a hard phase, and if a fraction of the polygonal ferrite is increased so the acicular ferrite is less than 60%, strength may deteriorate. Therefore, the area fraction of the acicular ferrite is 60% or more.

In addition, the inclusion of pearlite may lower tensile strength and low-temperature impact toughness, and thus, the microstructure of the steel of the present disclosure may not contain pearlite.

Here, the acicular ferrite measured in terms of the equivalent of a circle diameter is 30µm or less. If the size exceeds 30pm, impact toughness may be lowered.

Further, the bainite is granular bainite and upper bainite.

Meanwhile, an area fraction of the bainite is 30% or less. If the area fraction of the bainite exceeds 30%, an upper limit (440 MPa) of yield strength (440 MPa) which may cause ammonia stress corrosion cracking (SCC) may be exceeded, and thus, it is necessary to limit the fraction of the bainite.

The MA phase is 10% by area or less and the size measured by the equivalent of a circle diameter is preferably 5µm or less. MA (Martensite-Austenite constituent) is also referred to as a martensitic island.

If the fraction of the MA phase exceeds 10% or if the equivalent of a circle diameter exceeds 5µm, toughness of the base material and the welded portion tends to be significantly lowered. Therefore, it is necessary to limit the fraction and size of the MA phase.

Meanwhile, the steel of the present disclosure satisfying the above conditions may have a yield ratio (YS/TS) of 0.85 or less, preferably, 0.8 or less. The steel may have tensile strength of 490 MPa or greater, for example, about 510 to 610 MPa, having excellent tensile strength.

In addition, an upper limit of yield strength of the steel is 440 MPa or less and does not exceed the upper limit of yield strength which causes ammonia stress corrosion cracking (SCC), and thus, ammonia stress corrosion cracking (SCC) resistance may be excellent.

In addition, since an impact transition temperature of the 1/4t portion in a thickness direction of the steel is -60°C or lower, low temperature toughness may be excellent. Here t represents a thickness of the steel.

Here, the steel has a thickness of 6 mm or greater, and preferably, 6 to 50 mm.

As described above, the steel of the present disclosure may secure all of high strength, low yield ratio, excellent low temperature toughness, and ammonia stress corrosion cracking (SCC) resistance.

Hereinafter, a method for manufacturing a low yield ratio and high-strength steel having excellent stress corrosion cracking resistance and low temperature toughness according to another aspect of the present disclosure will be described in detail.

The method of manufacturing a low yield ratio and high-strength steel having excellent stress corrosion cracking resistance and low temperature toughness according to another aspect of the present disclosure includes : heating a slab having the above-described alloy composition to 1000 to 1200°C;
rough-rolling the heated slab at a temperature of 1100 to 900°C;
finishing-rolling at a temperature between Ar3 + 100°C and Ar3 + 30°C on the basis of a center temperature after the rough rolling; and
cooling to a temperature of 300°C or lower after the finishing-rolling.

### Heating

The slab having the above-described alloy composition is heated to 1000 to 1200°C.

The heating temperature of the slab is 1000°C or higher, and this is to dissolve a Ti carbonitride formed during casting. If the heating temperature of the slab is too low, deformation resistance during rolling is too high, so that a reduction ratio per rolling pass may not be increased in a follow-up rolling process, and thus, a lower limit thereof is limited to 1000°C. However, if heating is carried out at an excessively high temperature, austenite may be coarsened to lower toughness, and thus, an upper limit of the heating temperature is 1200°C.

### Rough rolling

The heated slab is subjected to rough rolling at a temperature of 1100 to 900°C.

The rough rolling temperature is set to be not lower than a temperature (Tnr) at which recrystallization of the austenite is stopped. An effect of breaking a cast structure such as dendrites formed during casting and reducing the size of austenite may be obtained through rolling. In order to obtain such an effect, the rough rolling temperature is limited to 1100 to 900°C.

Here, the rough rolling may be performed so that the last three rolling passes have a reduction ratio of 10% or greater per pass.

In order to provide sufficient deformation to the center during rough rolling, it is preferred that the reduction ratio per pass is at least 10% and a total cumulative reduction ratio is at least 30% for the last three rolling passes during rough rolling.

During rough rolling, grain growth is made in a recrystallized structure due to a high temperature in initial rolling, but when the last three rolling passes are performed, a grain growth rate is slowed as a bar is air-cooled in a rolling atmosphere, and due thereto, a reduction ratio of the last three passes during rough rolling most significantly affects a grain size of a final microstructure.

Also, if the reduction ratio per pass in rough rolling is lowered, sufficient deformation is not transferred to the central portion, which may cause toughness degradation due to center coarsening. Therefore, the reduction ratio per pass of the last three passes is preferably limited to 10% or greater.

Meanwhile, in order to miniaturize the structure at the central portion, it is preferable to set a cumulative rolling reduction ratio at the time of rough rolling to 30% or greater.

### Finishing rolling

After the rough rolling, finishing rolling is performed at a temperature between Ar3 + 100°C and Ar3 + 30°C on the basis of a temperature of the central portion.

This is to obtain a finer microstructure, and when finishing rolling is performed at Ar3 (ferrite transformation start temperature) + 100°C to Ar3 + 30°C, a large amount of deformation bands is generated in the austenite to secure a large amount of ferrite nucleation sites, obtaining an effect of securing a fine structure up to the central portion of the steel.

If the temperature for finishing rolling is lowered to below Ar3 + 30°C, the ferrite grain size becomes too fine to exceed the yield strength upper limit (440 MPa) causing ammonia stress corrosion cracking (SCC). Also, finishing rolling performed at a temperature exceeding Ar3 + 100°C is not effective in miniaturizing the grain size. Thus, the finishing rolling is carried out at a temperature between Ar3 +100°C and Ar3 +30°C and a microstructure of the steel sheet to be subjected to finishing rolling under such conditions may be a composite structure having the features mentioned above.

Here, the Ar3 is calculated as Ar3=910-(310^{∗}C)-(80^{∗}Mn)-(55^{∗}Ni), each element symbol represents the content of each element measured in wt%, and the unit of Ar3 is °C.

Further, in order to effectively generate a large amount of deformation bands in the austenite, it is more preferable to maintain the cumulative reduction ratio at 60% or greater during finishing rolling and to maintain the reduction ratio per pass, excluding the final shape sizing phase, at 10% or more .

### Cooling

After the finishing rolling, the steel sheet is cooled to a temperature of 300°C or lower.

After the finishing rolling, the cooling is started at a temperature of Ar3+30°C to Ar3 and cooled to a finish cooling temperature (FCT) of 300°C or lower, for example, about 100 to 300°C.

If the finish cooling temperature (FCT) is higher than 300°C, the fine MA phase may be decomposed due to a tempering effect to make it difficult to realize a low yield ratio. Thus, the finish cooling temperature is 300°C or lower.

Here, in performing cooling, first cooling is performed such that a cooling rate at the central portion is 15°C/s or greater up to Bs-10°C to Bs+10, and second cooling is performed up to 300°C or lower such that a cooling rate at the central portion is 10 to 50°C/s.

The cooling start temperature is Ar3 + 30°C to Ar3.

The above-mentioned first cooling starts, after finishing rolling, to perform cooling at a temperature of Ar3 + 30°C to Ar3 up to Bs-10°C at a cooling rate of 15°C/s or higher, for example, 30°C/s or higher, in the central portion of the steel sheet.

If the cooling rate of the central portion of the steel sheet is lower than 15°C/s up to Bs-10°C to Bs+10°C in the first cooling, it is possible to form a coarse polygonal ferrite to lower tensile strength and impact toughness.

Here, Bs is calculated as Bs=830-(270^{∗}C)-(90^{∗}Mn)-(37^{∗}Ni), each element symbol represents the content of each element measured in wt%, and the unit of Bs is °C.

The second cooling is performed after the first cooling up to the finish cooling temperature of 300°C or lower, for example, 100 to 300°C, at a cooling rate of 10°C/s to 50°C/s in the central portion of the steel sheet.

If the cooling rate of the steel sheet exceeds 50°C/s in the second cooling, the bainite fraction is formed to be 30% or greater by area as in the microstructure of 1- (1) of FIG. 1 to exceed the yield strength upper limit (440 MPa) causing ammonia stress corrosion cracking (SCC), and the excessive increase in strength may lower elongation and impact toughness .

Meanwhile, if the cooling rate of the steel sheet is lower than 10°C/s in the second cooling, a coarse polygonal ferrite and pearlite, rather than the fine acicular ferrite like the microstructure of 1-(3) of FIG. 1, may be formed, leading to a possibility that tensile strength is 490 MPa or less and Charpy transition temperature is -60°C or higher.

According to the above-described manufacturing method, it is possible to manufacture a low yield ratio and high-strength steel having excellent stress corrosion cracking resistance and low temperature toughness.

### [Mode for invention]

Hereinafter, the present disclosure will be described in detail by way of examples. It should be noted, however, that the following examples are intended to illustrate the present disclosure in more detail and not to limit the scope of the present disclosure and the scope of the present disclosure is determined by the matters described in the claims and the matters reasonably inferred therefrom.

A 300 mm-thick steel slab having the composition shown in Table 1 below was reheated to a temperature of 1100°C and then subjected to rough rolling at a temperature of 1050°C to prepare a bar. A cumulative reduction ratio during rough rolling was applied equally as 30%. Also, Ar3 and Bs temperatures according to compositions of each steel were calculated and are shown in Table 1 below.

After the rough rolling, finishing rolling was performed to satisfy the difference between the finishing rolling temperature and the Ar3 temperature shown in Table 2 below to obtain a steel sheet having the thickness shown in Table 2, and thereafter, cooling performed at various cooling rates through multistage cooling. Here, a finish cooling temperature of first cooling was equal to the Bs temperature of each steel.

The microstructure, yield strength, tensile strength, yield ratio, Charpy impact transition temperature, and ammonia stress corrosion cracking (SCC) test were performed on the steel sheet prepared as described above, and the results are shown in Table 3.

A sample of the microstructure was taken from the 1/4t portion of the steel sheet, mirror-polished, corroded using a Nital corrosion solution, and observed using an optical microscopy, and thereafter, a phase ratio was obtained through an image analysis.

A sample was taken from a 1/4t portion of the steel sheet, mirror-polished, corroded using a LePera corrosion solution, and observed using an optical microscope, and thereafter, a phase ratio of the MA phase was obtained through an image analysis.

A sample of No. JIS4 was taken from a 1/4t portion of the steel sheet in a direction perpendicular to a rolling direction and subjected to a tensile test at room temperature to measure yield strength, tensile strength and A yield ratio.

As for the low-temperature impact toughness, a sample was taken from a 1/4t portion of the steel sheet in a direction perpendicular to the rolling direction to manufacture a V-notch test sample and Charpy impact test was performed three times at each temperature at temperatures from -20 to -100°C at an internal of 20°C to derive a regression equation of each temperature average value, and low-temperature impact toughness was obtained at a temperature of 100J as a transition temperature.

In addition, the ammonia stress corrosion cracking (SCC) test was carried out using the test solution under the test conditions described in Table 4 by making proof ring test samples. 80% of actual yield stress was applied, and samples which were not broken for 720 hours were evaluated as pass and samples which were broken before 720 hours were evaluated as fail.

**[Table 1]**

| Steel type | Steel composition (wt%) | | | | | | | | | Ar₃ (°C) | Bs (°C) |
|---|---|---|---|---|---|---|---|---|---|---|---|
| | C | Si | Mn | Ni | Ti | Al | Nb | P (ppm) | S (ppm) | | |
| Inventive steel A | 0.08 | 0.3 | 1.5 | 0.2 | 0.01 | 0.03 | 0.003 | 59 | 25 | 754 | 666 |
| Inventive steel B | 0.072 | 0.27 | 1.32 | 0.34 | 0.012 | 0.024 | 0.001 | 46 | 31 | 763 | 679 |
| Comparative Steel C | 0.12 | 0.16 | 1.25 | 0.63 | 0.018 | 0.013 | 0.001 | 49 | 9 | 738 | 662 |
| Comparative Steel D | 0.062 | 0.32 | 2.11 | 0.65 | 0.011 | 0.026 | 0.002 | 55 | 17 | 686 | 599 |
| Comparative Steel E | 0.07 | 0.21 | 1.32 | 1.62 | 0.013 | 0.032 | 0.001 | 79 | 24 | 694 | 632 |
| Comparative Steel F | 0.069 | 0.23 | 1.41 | 0.52 | 0.021 | 0.033 | 0.035 | 81 | 33 | 747 | 665 |

**[Table 2]**

| Steel type | Classification | | Finishing rolling temperature -Ar₃ temperature (°C) | Product thickness (mm) | First cooling rate (°C/s) | Second cooling rate (°C/s) | Finish cooling temperature (°C) |
|---|---|---|---|---|---|---|---|
| Inventive steel A | A-1 | Inventive example | 45 | 20 | 40 | 45 | 250 |
| | A-2 | Comparative example | 150 | 20 | 38 | 25 | 280 |
| | A-3 | Comparative example | -30 | 20 | 35 | 30 | 150 |
| | A-4 | Comparative example | 30 | 30 | 8 | 15 | 240 |
| | A-5 | Comparative example | 18 | 15 | 50 | 75 | 150 |
| | A-6 | Comparative example | 50 | 35 | 15 | 7 | 300 |
| | A-7 | Comparative example | 50 | 35 | 15 | 25 | 450 |
| Inventive steel B | B-1 | Inventive example | 50 | 9 | 52 | 30 | 210 |
| | B-2 | Comparative example | 200 | 50 | 15 | 10 | 150 |
| | B-3 | Comparative example | -55 | 9 | 50 | 45 | 150 |
| | B-4 | Comparative example | 30 | 50 | 5 | 15 | 140 |
| | B-5 | Comparative example | 18 | 10 | 55 | 80 | 210 |
| | B-6 | Comparative example | 90 | 50 | 16 | 5 | 230 |
| | B-7 | Comparative example | 45 | 12 | 54 | 44 | 420 |
| Comparative Steel C | C-1 | Comparative example | 10 | 9 | 55 | 41 | 200 |
| Comparative Steel D | D-1 | Comparative example | 15 | 12 | 52 | 35 | 150 |
| Comparative Steel E | E-1 | Comparative example | 18 | 9 | 60 | 45 | 150 |
| Comparative Steel F | F-1 | Comparative example | 10 | 8 | 65 | 48 | 150 |

**[Table 3]**

| Steel type | Classification | | Microstructure phase fraction (area%) | | | | Yield strength (MPa) | Tensile strength (MPa) | Yield ratio | Impact transition temperature (°C) | Evaluation of Ammonia stress corrosion cracking (SCC) |
|---|---|---|---|---|---|---|---|---|---|---|---|
| | | | AF | B | PF | MA | | | | | |
| Inventive steel A | A-1 | Inventive example | 75 | 20 | 0 | 5 | 412 | 556 | 0.74 | -78 | Pass |
| | A-2 | Comparative example | 32 | 5 | 55 | 8 | 355 | 446 | 0.80 | -54 | Pass |
| | A-3 | Comparative example | 51 | 0 | 45 | 4 | 468 | 542 | 0.86 | -72 | Fail |
| | A-4 | Comparative example | 30 | 3 | 62 | 5 | 367 | 471 | 0.78 | -48 | Pass |
| | A-5 | Comparative example | 36 | 60 | 0 | 4 | 510 | 632 | 0.81 | -31 | Fail |
| | A-6 | Comparative example | 23 | 0 | 75 | 2 | 322 | 451 | 0.71 | -46 | Pass |
| | A-7 | Comparative example | 55 | 15 | 30 | 0 | 465 | 518 | 0.90 | -51 | Pass |
| Inventive steel B | B-1 | Inventive example | 80 | 12 | 0 | 8 | 424 | 563 | 0.75 | -90 | Pass |
| | B-2 | Comparative example | 34 | 12 | 50 | 4 | 326 | 451 | 0.72 | -44 | Pass |
| | B-3 | Comparative example | 50 | 0 | 48 | 2 | 459 | 512 | 0.90 | -95 | Fail |
| | B-4 | Comparative example | 35 | 5 | 58 | 2 | 325 | 425 | 0.76 | -32 | Pass |
| | B-5 | Comparative example | 20 | 77 | 0 | 3 | 583 | 642 | 0.91 | -65 | Fail |
| | B-6 | Comparative example | 25 | 0 | 70 | 5 | 333 | 423 | 0.79 | -62 | Pass |
| | B-7 | Comparative example | 32 | 36 | 32 | 0 | 486 | 521 | 0.93 | -65 | fail |
| Comparative Steel C | C-1 | Comparative example | 42 | 56 | 0 | 2 | 512 | 680 | 0.75 | -23 | fail |
| Comparative Steel D | D-1 | Comparative example | 30 | 68 | 0 | 2 | 543 | 625 | 0.87 | -36 | fail |
| Comparative Steel E | E-1 | Comparative example | 70 | 15 | 0 | 15 | 435 | 552 | 0.79 | -80 | fail |
| Comparative Steel F | F-1 | Comparative example | 78 | 2 | 15 | 5 | 556 | 612 | 0.91 | -90 | fail |

In Table 3, AF: Acicular Ferrite, B: Bainite, PF: Polygonal ferrite and MA: Martensite/Austenite.

**[Table 4]**

| Sample | Proof ring sample |
|---|---|
| Test solution | Liquefied ammonia |
| | 5 wt% of ammonium carbamate |
| | 0.1% of O₂ is contained |
| Test temperature | 25°C |
| Test time | 720 hours |

As shown in Tables 1 to 3, it can be seen that the inventive examples satisfying the compositions and manufacturing conditions proposed in the present disclosure are steel having excellent ammonia stress corrosion cracking (SCC) resistance, as well as having high strength and high toughness, and having a yield ratio of 0.8 or less, low yield ratio characteristics. Also, the microstructure of the inventive example A-1 was observed with a microscope and the results showed that the microstructure was a mixed structure including, in area %, 60% of more of acicular ferrite and the balance including at least one phase of bainite, polygonal ferrite and martensite-austenite constituent (MA) as illustrated in 1-(2) of FIG. 1.

Meanwhile, in the case of Comparative Examples A-2, A-4, A-6, B-2, B-4 and B-6 in which the compositions satisfied the present disclosure but manufacturing conditions did not satisfy the present disclosure, the polygonal ferrite fraction was too high or the ferrite grain size was too coarse to secure tensile strength and low temperature toughness.

Meanwhile, in the case of Comparative Examples A-3, A-5, A-7 to B-3, B-5 and B-7, the acicular ferrite grain size was too small or the bainite fraction was too high, or the MA phase was not produced, and thus, the yield strength upper limit (440 MPa) at which the ammonia stress corrosion cracking (SCC) may occur was exceeded to cause the ammonia stress corrosion cracking (SCC) and it was impossible to secure a low yield ratio and low temperature toughness.

Also, in the case of Comparative Examples C-1 to F-4 in which the manufacturing conditions satisfied the present disclosure but the compositions did not satisfy the present disclosure, the bainite fraction was too high, the acicular ferrite grain size was too small, or the fraction of MA phase was too high, and thus, the yield strength upper limit (440 MPa) at which the ammonia stress corrosion cracking (SCC) may occur was exceeded to cause the ammonia stress corrosion cracking (SCC) and it was impossible to secure a low yield ratio and low temperature toughness.

While example embodiments have been shown and described above, it will be apparent to those skilled in the art that modifications and variations could be made without departing from the scope of the present invention as defined by the appended claims.

## Claims

1. A low yield ratio and high-strength steel having excellent stress corrosion cracking resistance and low temperature toughness, comprising:
by weight percent, 0.02 to 0.10% of carbon (C), 0.5 to 2.0% of manganese (Mn), 0.05 to 0.5% of silicon (Si), 0.05 to 1.0% of nickel (Ni), 0.005 to 0.1% of titanium (Ti), 0.005 to 0.5% of aluminum (Al), 0.003% or less of niobium (Nb), 0.015% or less of phosphorus (P), 0.015% or less of sulfur (S), a balance of Fe and other inevitable impurities,
wherein a microstructure includes, in area percent (%), 60% or more of acicular ferrite and the balance including at least one phase of bainite, polygonal ferrite and martensite-austenite constituent (MA),
wherein a size of the acicular ferrite measured in terms of the equivalent of a circle diameter is 30µm or less,
wherein the bainite has a 30 area% or less,
wherein the MA phase is 10 area% or less and
wherein the steel has a thickness of 6 mm or greater. The measurement methods of all claimed parameters are disclosed in the description.

2. The steel of claim 1, wherein a size of the MA phase measured in terms of the equivalent of a circle diameter is 5µm or less.

3. The steel of claim 1, wherein a yield ratio of the steel is 0.85 or less and tensile strength of the steel is 490 MPa or greater. The measurement method for the tensile strength is described in the description.

4. The steel of claim 1, wherein yield strength of the steel is 440 MPa or less. The measurement method for the yield strength described in the description.

5. The steel of claim 1, wherein an impact transition temperature of the steel is -60°C or lower. The measurement method for impact transition temperature described in the description.

6. A method of manufacturing a low yield ratio and high-strength steel having low temperature toughness according to claim 1 the method comprising:
heating a slab including, by weight percent, 0.02 to 0.10% of carbon (C), 0.5 to 2.0% of manganese (Mn), 0.05 to 0.5% of silicon (Si), 0.05 to 1.0% of nickel (Ni), 0.005 to 0.1% of titanium (Ti), 0.005 to 0.5% of aluminum (Al), 0.003% or less of niobium (Nb), 0.015% or less of phosphorus (P), 0.015% or less of sulfur (S), a balance of Fe and other inevitable impurities, to 1000 to 1200°C;
rough-rolling the heated slab at a temperature of 1100 to 900°C;
finishing-rolling at a temperature between Ar3 + 100°C and Ar3 + 30°C on the basis of a center temperature after the rough rolling; and
cooling to a temperature of 300°C or lower after the finishing-rolling,
wherein in performing cooling, first cooling is performed such that a cooling rate at the central portion is 15°C/s or greater up to Bs-10°C to Bs+10°C and
second cooling is performed up to 300°C or lower such that a cooling rate at the central portion is 10 to 50°C/s.
Ar3 and Bs are calculated as follows: $Ar 3 = 910 - \left(310*C\right) - \left(80*N\right) - \left(55*Ni\right) ;$ $Bs = 830 - \left(270*C\right) - \left(90*Mn\right) - \left(37*Ni\right)$

7. The method of claim 6, wherein a cooling start temperature is Ar3 + 30°C to Ar3.

8. The method of claim 6, wherein the rough rolling is performed so that the last three rolling passes have a reduction ratio of 10% or greater per pass.

9. The method of claim 6, wherein the finishing rolling is performed such that a reduction ratio per pass is 10% or greater and a cumulative reduction ratio is 60% or greater.

## Patentansprüche

1. Niedriges Streckgrenzenverhältnis und hochfester Stahl mit ausgezeichneter Spannungsrisskorrosionsbeständigkeit und Tieftemperaturzähigkeit, Folgendes umfassend:
in Gewichtsprozent, 0,02 bis 0,10 % Kohlenstoff (C), 0,5 bis 2,0 % Mangan (Mn), 0,05 bis 0,5 % Silizium (Si), 0,05 bis 1,0 % Nickel (Ni), 0,005 bis 0,1 % Titan (Ti), 0,005 bis 0,5 % Aluminium (Al), 0,003 % oder weniger Niob (Nb), 0,015 % oder weniger Phosphor (P), 0,015 % oder weniger Schwefel (S), Rest an Fe und andere unvermeidliche Verunreinigungen, wobei eine Mikrostruktur in Flächenprozent (%) 60 % oder mehr an nadelförmigem Ferrit enthält und der Rest mindestens eine Phase aus Bainit, polygonalem Ferrit und Martensit-Austenit-Bestandteil (MA) enthält, wobei eine Größe des nadelförmigen Ferrits, gemessen als Äquivalent eines Kreisdurchmessers, 30 µm oder weniger beträgt, wobei der Bainit 30 Flächen-% oder weniger aufweist, wobei die MA-Phase 10 Flächen-% oder weniger beträgt und wobei der Stahl eine Dicke von 6 mm oder mehr aufweist. Die Messmethoden aller beanspruchten Parameter sind in der Beschreibung offenbart.

2. Stahl nach Anspruch 1, wobei die Größe der MA-Phase, gemessen als Äquivalent eines Kreisdurchmessers, 5 µm oder weniger beträgt.

3. Stahl nach Anspruch 1, wobei das Streckgrenzenverhältnis des Stahls 0,85 oder weniger und die Zugfestigkeit des Stahls 490 MPa oder mehr beträgt. Die Messmethode für die Zugfestigkeit ist in der Beschreibung beschrieben.

4. Stahl nach Anspruch 1, wobei die Streckgrenze des Stahls 440 MPa oder weniger beträgt. Die Messmethode für die Streckgrenze ist in der Beschreibung beschrieben.

5. Stahl nach Anspruch 1, wobei die Kerbschlagzähigkeitsübergangstemperatur des Stahls - 60 °C oder niedriger ist. Die Messmethode für die Kerbschlagzähigkeitsübergangstemperatur ist in der Beschreibung beschrieben.

6. Verfahren zur Herstellung eines niedrigen Streckgrenzenverhältnisses und eines hochfesten Stahls mit Tieftemperaturzähigkeit nach Anspruch 1, wobei das Verfahren Folgendes umfasst:
Erhitzen einer Bramme mit folgenden Bestandteilen in Gewichtsprozent: 0,02 bis 0,10 % Kohlenstoff (C), 0,5 bis 2,0 % Mangan (Mn), 0,05 bis 0,5 % Silizium (Si), 0,05 bis 1,0 % Nickel (Ni), 0,005 bis 0,1 % Titan (Ti), 0.005 bis 0,5 % Aluminium (Al), 0,003 % oder weniger Niob (Nb), 0,015 % oder weniger Phosphor (P), 0,015 % oder weniger Schwefel (S), Rest an Fe und andere unvermeidliche Verunreinigungen, bis 1000 bis 1200 °C;
Vorwalzen der erhitzten Bramme bei einer Temperatur von 1100 bis 900 °C;
Fertigwalzen bei einer Temperatur zwischen Ar3 + 100 °C und Ar3 + 30°C auf der Basis einer Mittentemperatur nach dem Vorwalzen; und
Abkühlen auf eine Temperatur von 300 °C oder niedriger nach dem Fertigwalzen, wobei bei der Durchführung des Abkühlvorgangs eine erste Abkühlung so durchgeführt wird, dass eine Abkühlgeschwindigkeit im zentralen Abschnitt 15 °C/s oder mehr bis zu Bs-10 °C bis Bs+10 °C beträgt, und eine zweite Abkühlung bis zu 300 °C oder niedriger durchgeführt wird, so dass eine Abkühlgeschwindigkeit im zentralen Abschnitt 10 bis 50 °C/s beträgt.
Ar3 und Bs werden wie folgt berechnet: $Ar 3 = 910 - \left(310*C\right) - \left(80*N\right) - \left(55*Ni\right) ;$ $Bs = 830 - \left(270*C\right) - \left(90*Mn\right) - \left(37*Ni\right)$

7. Verfahren nach Anspruch 6, wobei die Anfangstemperatur beim Abkühlen Ar3 + 30 °C bis Ar3 beträgt.

8. Verfahren nach Anspruch 6, wobei das Vorwalzen so durchgeführt wird, dass die letzten drei Walzdurchläufe ein Reduktionsverhältnis von 10 % oder mehr pro Durchlauf aufweisen.

9. Verfahren nach Anspruch 6, wobei das Fertigwalzen so durchgeführt wird, dass ein Reduktionsverhältnis pro Durchgang 10 % oder mehr und ein kumulatives Reduktionsverhältnis 60 % oder mehr beträgt.

## Revendications

1. Acier à faible rapport d'élasticité et à haute résistance présentant une excellente résistance à la fissuration par corrosion sous contrainte et une ténacité à basse température, comprenant :
en pourcentage en poids, 0,02 à 0,10 % de carbone (C), 0,5 à 2,0 % de manganèse (Mn), 0,05 à 0,5 % de silicium (Si), 0,05 à 1,0 % de nickel (Ni), 0,005 à 0,1 % de titane (Ti), 0,005 à 0,5 % d'aluminium (Al), au plus 0,003 % de niobium (Nb), au plus 0,015 % de phosphore (P), au plus 0,015 % de soufre (S), un complément de Fe et d'autres impuretés inévitables,
dans lequel une microstructure comprend, en pourcentage de surface (%), au moins 60 % de ferrite aciculaire et le complément comprenant au moins une phase de bainite, de ferrite polygonale et de martensite-austénite (MA),
dans lequel une taille de ferrite aciculaire mesurée en termes d'équivalent d'un diamètre de cercle est d'au plus 30 µm,
dans lequel la bainite a au plus 30 % en surface,
dans lequel la phase MA est d'au plus 10 % en surface, et dans lequel l'acier a une épaisseur d'au moins 6 mm.
Les procédés de mesure de tous les paramètres revendiqués sont présentés dans la description.

2. Acier selon la revendication 1, dans lequel une taille de la phase MA mesurée en termes d'équivalent d'un diamètre de cercle est d'au plus 5 µm.

3. Acier selon la revendication 1, dans lequel un rapport d'élasticité de l'acier est d'au plus 0,85 et où la résistance à la traction de l'acier est d'au moins 490 Mpa, le procédé de mesure de la résistance à la traction étant présenté dans la description.

4. Acier selon la revendication 1, dans lequel la limite d'élasticité de l'acier est d'au plus 440 MPa. Le procédé de mesure de la limite d'élasticité est présenté dans la description.

5. Acier selon la revendication 1, dans lequel une température de transition d'impact de l'acier est d'au plus -60 °C.
Le procédé de mesure de la température de transition d'impact est présenté dans la description.

6. Procédé de production d'un acier à faible rapport d'élasticité et à haute résistance présentant une ténacité à basse température selon la revendication 1, le procédé comprenant :
le chauffage d'une dalle comprenant, en pourcentage en poids, 0,02 à 0,10 % de carbone (C), 0,5 à 2,0 % de manganèse (Mn), 0,05 à 0,5 % de silicium (Si), 0,05 à 1,0 % de nickel (Ni), 0,005 à 0,1 % de titane (Ti), 0,005 à 0,5 % d'aluminium (Al), au plus 0,003 % de niobium (Nb), au plus 0,015 % de phosphore (P), au plus 0,015 % de soufre (S), un complément de Fe et d'autres impuretés inévitables, à 1 000 à 1 200 °C ;
le laminage grossier de la dalle chauffée à une température de 1 100 à 900 °C ;
le laminage de finition à une température comprise entre Ar3 + 100 °C et Ar3 + 30 °C en fonction d'une température centrale après le laminage grossier ; et
le refroidissement à une température d'au plus 300 °C après le laminage de finition, et lors du refroidissement, le premier refroidissement est effectué de telle manière qu'une vitesse de refroidissement au niveau de la partie centrale soit d'au moins 15 °C/s jusqu'à Bs - 10 °C à Bs + 10 °C et un second refroidissement est effectué jusqu'à au plus 300 °C, de sorte qu'une vitesse de refroidissement au niveau de la partie centrale soit de 10 à 50 °C/s.
Ar3 et Bs sont calculés comme suit : $Ar 3 = 910 - \left(310*C\right) - \left(80*N\right) - \left(55*Ni\right) ;$ $Bs = 830 - \left(270*C\right) - \left(90*Mn\right) - \left(37*Ni\right)$

7. Procédé selon la revendication 6, dans lequel une température de début de refroidissement est Ar3 + 30 °C à Ar3.

8. Procédé selon la revendication 6, dans lequel le laminage grossier est effectué de telle manière que les trois dernières passes de laminage aient un taux de réduction d'au moins 10 % par passe.

9. Procédé selon la revendication 6, dans lequel le laminage de finition est effectué de telle manière qu'un taux de réduction par passe soit d'au moins 10 % et qu'un taux de réduction cumulé soit d'au moins 60 %.
